

# UNITED STATES PATENT OFFICE.

ERNST VOETTER, OF KREFELD, NEAR BOCKUM, GERMANY.

## PREPARING COMPOUNDS OF CHROMIUM OXID.

1,228,622.

Specification of Letters Patent.

Patented June 5, 1917.

No Drawing.

Application filed July 2, 1914. Serial No. 848,561.

*To all whom it may concern:*

Be it known that I, ERNST VOETTER, chemist, a subject of the King of Wurttemberg and the German Emperor, residing at Bockumerplatz 2, Krefeld, near Bockum, Kingdom of Prussia, German Empire, have invented a new and useful Improvement in Preparing Compounds of Chromium Oxid; and I do hereby declare the following to be a full, clear, and exact description of the same.

The conversion of chromic acid or chromates into lower oxidation stages is commonly effected by the action of glucose in the presence of acids, whereupon a strong reaction sets in and a chromium salt of the acid is obtained, *e. g.* chromium sulfate.

These chromium solutions may be used either immediately or first neutralized with alkalies or salts of organic acids, as sodium acetate, or else solutions of hydrated chromium oxid are formed by the action of sodium hydrate solution. These chromium compounds are extensively used as tanning and mordanting agents.

It is now found that under certain conditions chromic acid and chromates can be reduced without an addition of acid, indeed even in an alkaline solution. In neutral solutions, insoluble hydrated chromium oxid is obtained in the form of black shining grains which dissolve readily in acid with the evolution of gas. In alkaline solution, soluble complex basic chromium compounds are formed which may be converted into salts of any basicity by the addition of acids.

The water-insoluble hydrated chromium oxid found by me is produced by the action of glucose on acid chromates and chromic acid, in some cases with an addition of thiosulfate. When employing chromic acid, the reaction sets in with glucose without the aid of heat, but when employing acid dichromates and glucose the mixtures must be brought nearly to the boiling point. If, however, thiosulfate is added, the reaction takes place at a considerably lower temperature. The stable chromium compound thus produced is in the form of black shining grains. This body contains chromium hy-

droxid, carbonic acid chemically combined, organic acids of the aliphatic series and aldehydes of the aliphatic series. An exact formula cannot be given for the compounds because the relative proportion of the components varies. The compound is particularly adapted for tanning purposes.

Furthermore, I have found that when reducing chromates with glucose, for instance, in the presence of ammonia, *i. e.* in a weakly alkaline solution, a water-insoluble hydrated chromium oxid is obtained. Ammonia may be partly replaced by sodium carbonate, and glucose likewise by thiosulfate.

It was then found that by reducing chromates with glucose or other sorts of sugar in a neutral or weakly caustic alkaline solution basic chromium carbonate in the soluble form results. The liquid obtained is green, thick, syrupy and readily soluble in water. It is a matter of surprise that acid may be added to the solution until it reacts perfectly neutral, without precipitation taking place, the solution remaining perfectly clear until a small excess of acid precipitates hydrated chromium oxid which, with a further addition of acid, readily dissolves in the cold. In this way, normal or more or less basic salts are obtained, which may be immediately employed for tanning and mordanting.

The production is very simple. Either neutral chromate is used or chromic acid or dichromates are converted into the neutral, yellow salt by an addition of alkalies, as sodium hydrate solution or sodium carbonate, adding if necessary, a small excess of alkali and then the necessary quantity of either grape sugar alone or grape sugar and thio-sulfate.

Normal salts, basic salts and neutral solutions of chromium oxid can be produced *ad libitum* from these new chromium compounds, so that these compounds can be extensively employed for any purpose of tanning and mordanting.

For certain purposes the process may also be carried out upon organic or inorganic solid substances, such as textile fibers, leather, china clay, the new chromium com-

pounds being immediately fixed on said substances in the very moment of their formation.

According to the purpose for which it is to be employed, the chromic acid may be only partially reduced, the result being a mixture of chromates and chromium salts.

*Example.*

10 1. Dissolve 82 kg. sodium dichromate in  
78 lt. water, add  
40 " 4:5 glucose solution  
and  
22 kg. thiosulfate

15 and warm to 70-80° C., at which temperature reaction sets in. Without any further introduction of heat, the temperature rises to 110° C. Much gas evolves and a porous, black-shining product is formed, which may be used immediately or cleansed by washing in water.

As an example for producing a solution therefrom, a mixture of

25 100 lt. sulfuric acid 60° C. and  
50 " water is poured over  
260 kg. of the crude product.

Solution takes place gradually with the evolution of much heat, and gas consisting chiefly of carbon dioxide mixed with small amounts of carbon monoxide; and the result is a highly concentrated chromium extract of 60° B., which may be used for tanning and mordanting, either immediately or after being neutralized with sodium carbonate or salts of inorganic acids, *e. g.* sodium acetate.

40 2. Dissolve 82.5 kg. sodium dichromate  
and  
60.0 kg. solid glucose in  
67.5 lt. water at about 90° C.,  
adding gradually  
45 50.0 lt. of 20 per cent. ammonia.

After a short time, much gas is evolved, and black-shining grains are formed, which may be used as stated in example No. 1.

50 3. Dissolve 82.0 kg. sodium dichromate  
in  
68.0 lt. water, add  
48-50 " sodium hydrate solution  
55 at 40° B. and then  
80 lt. 1:1 glucose solution.

When the mixture is brought to 80° C., much gas is evolved, and the temperature increases. The reaction ceases after a short time, and the result is a bright green syrup-like liquid which gives a clear solution in cold water.

4. Dissolve 89.4 kg. sodium chromate in  
80.0 lt. water, add  
40.0 " 4:5 glucose solution 65  
and finally  
22.0 kg. thiosulfate.

When brought to about 80° C., a strong reaction sets in, and the result is a syrup-like green liquid which readily dissolves in water.

5. Dissolve 55 kg. chromic acid in  
66 lt. water and add gradually  
75 40 lt. 4:5 glucose solution.

The temperature rises and gas is evolved, the result being a porous, black-shining product.

The above-stated quantities may be altered according to requirements.

I claim as my invention:

1. Process of preparing organic chromium compounds especially well adapted for tanning purposes, which consists in reducing compounds containing chromic acid with sugars in the absence of free acid other than chromic acid.

2. Process of preparing organic compounds of chromium oxide, which consists in reducing dichromates with sugars in the absence of free acid.

3. Process of preparing organic chromium compounds which consists in reducing compounds containing chromic acid with glucose in absence of free acids other than chromic acid.

4. Process of preparing organic chromium compounds which consists in reducing salts of chromic acid with glucose.

5. Process of preparing organic chromium compounds which consists in reducing salts of chromic acid with glucose and thiosulfate.

6. Process of preparing organic chromium compounds which consists in reducing compounds containing chromic acid with glucose in absence of free acids different from chromic acid and converting the obtained compounds into soluble chromium salts by the action of acids.

7. Process of preparing organic chromium compounds which consists in reducing salts of chromic acid with glucose and converting the obtained compounds into soluble chromium salts by the action of acids.

In testimony whereof, I have signed my name to this specification in the presence of two subscribing witnesses.

ERNST VOETTER.

Witnesses:

PAUL DREES,  
HENRY QUADFLIEG.